

## 1

2,816,869

## SEMI-FLUID LUBRICANT

Paul R. McCarthy, Allison Park, Pa., assignor to Gulf Research & Development Company, Pittsburgh, Pa., a corporation of Delaware

No Drawing. Application May 29, 1956,  
Serial No. 587,966

5 Claims. (Cl. 252—57)

This invention relates to an improved semi-fluid lubricant and more particularly to a thixotropic lubricating composition having high adhesive properties in the liquid state.

In certain types of lubrication there are encountered conditions under which neither greases nor liquid oils are entirely satisfactory lubricants. For example, in the lubrication of certain textile machinery such as plain bearings on looms, top rolls, roll necks and saddles of drawing, roving and spinning frames, it is desirable that the lubricant be of such consistency that it will remain between the working surfaces and not be lost by dripping, leakage or centrifugal force. At the same time, it is desirable that the lubricant be of relatively low viscosity under operating conditions so as to neither impede the operation of the mechanism nor increase the power consumption.

Employing a textile-machinery lubricant which will stay on the bearing surface is important not only from the standpoint of the life of the bearing, but also from the standpoint of the product of the mill. Obviously, lubrication failure of the bearing will result in costly shut-down of the machinery. Also, leakage of lubricant onto the product of the mill, whether thread or woven fabric, will result in undesirable staining of the fabric.

In addition to the above requirements the textile machinery lubricant must feed through wicks without clogging and must be dispensable from ordinary "squirt-type" oil cans. While liquid oils can be dispensed from oil cans and are generally satisfactory lubricants, as a general rule they do not have good metal adhesion properties. Greases have good metal adhesion properties but are undesirable in that they can not be applied by wick feed or by ordinary oil cans.

Semi-fluid oils of the soap thickened type have been extensively used for lubricating textile machinery. Soap-thickened lubricants, however, have certain shortcomings in that frequently lumps of soap appear which clog the wicks. The soap-thickened lubricants have also been undesirable in that lubricants having identical properties are difficult to reproduce. Furthermore, soap-thickened lubricants having suitable adhesive properties, as a general rule, have some unsatisfactory property such as being stringy.

It is, therefore, an object achieved by this invention to provide an easily reproducible lubricating composition which will be sufficiently fluid to apply from an ordinary squirt-type oil can and will remain fluid while the bearings on which it is placed are in operation but will form a light gel when the bearings are not in operation.

This and other objects achieved by this invention will become apparent from the following detailed discussion.

I have discovered that a semi-fluid oil having thixotropic characteristics and improved metal adhesion in the liquid state can be prepared from a high viscosity hydrocarbon oil by compounding therewith small amounts of each of polymerized ethylene and a hydrogenated rosin. The

## 2

semi-fluid composition of the invention, since it does not rely upon soap as a gelling agent, is to be distinguished from greases insofar as the mode of obtaining a gel consistency is concerned.

- 5 The hydrocarbon oil employed in the preparation of the thixotropic composition according to this invention can be either a refined or semi-refined paraffinic, naphthenic, or asphalt-base oil, or the oil can be a synthetic oil having a viscosity above about 400 SUS at 100° F. and preferably having a viscosity of about 400 to 4000 SUS at 100° F. If desired, a blend of oils of suitable viscosity can be employed instead of a single oil, by means of which any desired viscosity within the range of 400 to 4000 SUS at 100° F. can be secured. The amount of oil employed constitutes from about 90 to 99 percent by weight of the total composition. Naturally, the optimum amount of oil employed in any given instance will depend upon the particular oil employed as well as upon the characteristics desired in the final composition.
- 10 The polymerized ethylene is a polymerization product of ethylene having a molecular weight of about 1000 to 40,000 or more. Polyethylenes having a molecular weight within this range, i. e., 19,000, are characterized by the following approximate characteristics:
- 15 Softening point, °C.----- 108  
Tensile strength, p. s. i----- 1200  
Yield point, p. s. i----- 1450
- 20 These polymerized ethylene compounds are obtained by the thermal or catalytic polymerization of ethylene at high pressure. The method of forming the polymers is not a part of the present invention. The amount of polymerized ethylene employed constitutes about 0.2 to about 5 percent by weight of the total composition.
- 25 The hydrogenated rosin employed according to the invention is a rosin of at least about 40 percent saturation to and including fully hydrogenated rosin. Rosin, sometimes called colophony, is the residue obtained on distilling turpentine from hard pine resin. Abietic acid,  $C_{20}H_{30}O_2$ , is the chief constituent of rosin and is obtained from the latter by distillation. Abietic acid is a carboxylic acid containing two double bonds. Hydrogenated rosin is obtained by the addition of hydrogen to the double bonds of abietic acid. The amount of hydrogen added may be sufficient to saturate the two unsaturated bonds of abietic acid or it may be any amount to produce substantial partial hydrogenation. A particularly useful hydrogenated rosin for the purposes of my invention is one which has been hydrogenated to about 50 to about 60 percent of capacity and has a melting point of about 168° F. The quantity of the hydrogenated rosin employed constitutes from about 0.2 to about 5 percent by weight of the total composition. In general, improved metal adhesion characteristics are obtained when the weight ratio of the hydrogenated rosin to the polymerized ethylene is between about 1:3 and about 3:1. In any event the mixture of hydrogenated rosin and polymerized ethylene is added in an amount sufficient to increase the viscosity of the hydrocarbon oil and to impart thixotropic characteristics thereto.
- 30
- 35
- 40
- 45
- 50
- 55
- 60

In preparing the improved lubricant of my invention I can also incorporate in the lubricant one or more of the so-called addition agents normally added to lubricating oils for a specific purpose including an anti-oxidant, a corrosion inhibitor, an anti-rust agent, an extreme pressure agent, an anti-foam agent and an oiliness agent. Corrosion inhibitors are particularly desirable in compositions used in corrodible alloy bearings. Among the corrosion inhibitors suitable for the purpose of the invention are dibenzyl disulfide, alkyl phenyl sulfides,

alkyl phosphites, alkaryl phosphites and sulfurized terpenes. In instances where the lubricant is subjected to prolonged use under oxidizing conditions, I advantageously incorporate in the lubricant a small amount of an oxidation inhibitor such as an alkali insoluble phenol, i. e., 2,6-di-tertiary-butyl-4-methylphenol; 2,4,6-tri-tertiary-butylphenol; etc., and/or a small amount of a diaryl amine. As examples of some of the diaryl amines which can be used in the composition of the invention may be mentioned diphenylamine, phenyl alpha naphthylamine, phenyl beta naphthylamine, alpha alpha-, alpha beta-, and beta beta-, dinaphthylamines, and the like. The amount of the conventional additive agents employed will depend to a large extent upon the conditions to which the composition is subjected, as well as upon the particular additive used. For instance, when the composition is subjected to prolonged use under oxidizing conditions, such as under extreme pressure and temperature, the oxidation inhibitor and extreme pressure agent requirements will be much greater than when relatively mild operating conditions are encountered. Generally, the amount of the anti-oxidant employed is between about 0.1 and 1.5 percent by weight based upon the weight of the total composition. In any event, the amount of additive employed is sufficient to accomplish the purpose for which it is intended without deleteriously affecting the other desirable characteristics of the composition.

In compounding the semi-fluid lubricant of the invention, various compounding and blending procedures can be used. In accordance with one embodiment, the hydrogenated rosin is placed in a vessel and then heated until it is liquid. The temperature thus attained is about 200° F. The polymerized ethylene is then added with stirring to the melted hydrogenated rosin while continuing to heat to 450° F. The mixture is then held at 450° F. for a time sufficient to effect a uniform dispersion. The time required depends upon the size of the batch as well as the efficiency of the dispersing means. An oil concentrate of the hydrogenated rosin-polymerized ethylene dispersion is then prepared by adding an amount of oil equivalent to the combined weight of the hydrogenated rosin and polymerized ethylene. Heating at 450° F. with stirring is continued until a uniform concentrate is obtained. The concentrate is then added to the base oil having the desired viscosity at 240° F. Stirring is continued to obtain a uniform blend. The mixture is then cooled to room temperature with or without stirring depending upon the viscosity desired in the final product. I have found that cooling without stirring from 240° F. to room temperature results in a product having a higher viscosity than a similar product which has been cooled from 240° F. to 120° F. with stirring. If a conventional additive such as an anti-oxidant is employed, it can be added to the dispersion of polymerized ethylene and hydrogenated rosin, or it can be added to the oil prior to the preparation of the concentrate. Of course, other compounding means can be employed without deviating from the scope of the invention.

The advantageous properties obtained by incorporating hydrogenated rosin and polymerized ethylene in a 750/4.5 Texas mineral oil as compared with the oil itself will be illustrated in connection with a metal adhesion test which is indicative of the adhesion characteristics obtainable in commercial application of a lubricant.

The metal adhesion test employed in comparing the lubricating compositions is that test ordinarily employed in determining the adhering characteristics of a grease. In conducting the test, a polished brass or steel disc with a concave surface is mounted on a vertical motor shaft so that the plane of the disc is in a horizontal position. The disc is tared. One tenth gram of lubricant is placed on the disc. The disc plus the lubricant is then reweighed. The disc is then attached to the motor shaft. The entire disc is encased in a closed chamber the temperature of

which is thermostatically controlled. The motor is then run for a period of seven minutes at a selected speed of 200 to 1000 R. P. M. at a selected temperature of 80° to 200° F. At the end of the seven-minute period, the disc plus lubricant is reweighed and the lubricant remaining on the disc is calculated as percent lubricant retention.

In preparing the following compositions, a lubricating oil having a viscosity of about 750 SUS at 100° F. was prepared by mixing 68 parts by volume of a Texas oil having a viscosity of about 500 SUS at 100° F. with 32 parts by volume of a Texas oil having a viscosity of about 1900 SUS at 100° F. Various amounts of polymerized ethylene and hydrogenated rosin were employed as shown. The polymerized ethylene was a solid having a molecular weight of about 19,000. The hydrogenated rosin employed was a solid having a melting point of about 168° F. The double bonds of the rosin acids had been saturated to an extent of about 50 to 60 percent. The blending procedure employed in preparing the compositions was in accordance with the embodiment described hereinabove. In preparing these compositions the rate of cooling from 240° to 120° F. was increased by stirring. Cooling from 120° F. to room temperature was without stirring.

Table 1

|                                                                                                                                   | A   | B     | C     | D     |
|-----------------------------------------------------------------------------------------------------------------------------------|-----|-------|-------|-------|
| Composition, percent by wt.:                                                                                                      |     |       |       |       |
| 750/4.5 Texas oil.....                                                                                                            | 100 | 98    | 98.5  | 99    |
| Hydrogenated rosin.....                                                                                                           |     | 1.332 | 1.0   | 0.668 |
| Polymerized ethylene.....                                                                                                         |     | 0.668 | 0.5   | 0.334 |
| Ratio of Hydrogenated rosin to<br>Polymerized ethylene.....                                                                       |     | 2:1   | 2:1   | 2:1   |
| Inspection:                                                                                                                       |     |       |       |       |
| Viscosity, SUS—                                                                                                                   |     |       |       |       |
| at 100° F.....                                                                                                                    | 753 | 1,597 | 1,228 | 1,153 |
| at 210° F.....                                                                                                                    | 62  | 80.4  | 74.4  | 70.3  |
| Adhesion to metal, percent re-<br>tained (0.1 gm. of lubricant<br>applied to disc rotated for 7<br>minutes at room temperature) — |     |       |       |       |
| at 200 R. P. M.....                                                                                                               | 100 | 100   | 100   | 100   |
| at 400 R. P. M.....                                                                                                               | 50  | 100   | 90    | 90    |
| at 600 R. P. M.....                                                                                                               | 40  | 80    | 70    | 60    |
| at 800 R. P. M.....                                                                                                               | 30  | 60    | 45    | 35    |
| at 1000 R. P. M.....                                                                                                              | 40  |       |       |       |
| Adhesion to metal, percent re-<br>tained (400 R. P. M.) —                                                                         |     |       |       |       |
| at 80° F.....                                                                                                                     | 63  | 98    | 97    | 85    |
| at 120° F.....                                                                                                                    | 65  | 100   | 95    | 100   |
| at 160° F.....                                                                                                                    | 45  | 93    | 93    | 88    |

It can be seen from the data in the above table that compositions B, C and D containing from 1 to 2 percent by weight of a mixture of hydrogenated rosin and polymerized ethylene in a 2 to 1, respectively, weight ratio gave remarkably improved metal adhesion characteristics. In the first series of tests, the temperature was maintained constant while varying the speed between 200 and 1000 R. P. M. In the second series of tests, the speed was maintained constant while varying the temperature between 80° and 160° F. In each series of tests, the compositions of the invention were strikingly superior.

The results of additional tests employing a composition containing two percent by weight of a mixture of hydrogenated rosin and polymerized ethylene in ratios between 1:3 and 3:1 are shown in Table 2. These compositions were prepared by the same procedure used in preparing the compositions reported in Table 1.

The data in Table 2 again show the improved metal adhesion characteristics of compositions within the scope of the invention. It will be noted that compositions B, C and E wherein the ratio of hydrogenated rosin to polymerized ethylene is 1:3, 1:2 and 2:1, respectively, gave particularly good retention of the lubricant at temperatures of 80° to 160° F.

As disclosed hereinabove, I have found that cooling without stirring from 240° F. to room temperature results in a product having a higher viscosity. This point

Table 2

|                                                     | A   | B     | C     | D     | E     | F     |
|-----------------------------------------------------|-----|-------|-------|-------|-------|-------|
| Composition, percent by wt.:                        |     |       |       |       |       |       |
| 750/4.5 Texas oil                                   | 100 | 98    | 98    | 98    | 98    | 98    |
| Hydrogenated rosin                                  |     | 0.48  | 0.66  | 1.0   | 1.34  | 1.52  |
| Polymerized ethylene                                |     | 1.52  | 1.34  | 1.0   | 0.66  | 0.48  |
| Ratio of Hydrogenated rosin to Polymerized ethylene |     | 1:3   | 1:2   | 1:1   | 2:1   | 3:1   |
| Inspection:                                         |     |       |       |       |       |       |
| Viscosity, SUS—                                     |     |       |       |       |       |       |
| at 100° F.                                          | 753 | 2,630 | 2,340 | 1,118 | 1,597 | 1,326 |
| at 210° F.                                          | 62  | 88    | 86.5  | 80.2  | 80.4  | 70.5  |
| Adhesion to metal, percent retained (400 R. P. M.)— |     |       |       |       |       |       |
| at 80° F.                                           | 63  | 100   | 100   | 93    | 98    | 100   |
| at 120° F.                                          | 65  | 100   | 100   | 90    | 100   | 89    |
| at 160° F.                                          | 45  | 100   | 100   | 81    | 93    | 73    |

can be illustrated by inspecting the viscosities of lubricating compositions which contain the same proportions of hydrogenated rosin and polymerized ethylene, the only difference being the manner in which cooling is effected. In Table 3, the compositions were prepared according to the blending procedure described hereinabove. After uniform blends were obtained, compositions A and C were cooled from 240° F. to room temperature without stirring; compositions B and D were cooled from 240° to 120° F. with stirring and then to room temperature without stirring.

Table 3

|                                                     | A     | B     | C     | D     |
|-----------------------------------------------------|-------|-------|-------|-------|
| Composition, percent by wt.:                        |       |       |       |       |
| 750/4.5 Texas oil                                   | 98    | 98    | 98    | 98    |
| Hydrogenated rosin                                  | 1.332 | 1.352 | 1     | 1     |
| Polymerized ethylene                                | 0.668 | 0.668 | 1     | 1     |
| Ratio of Hydrogenated rosin to Polymerized ethylene | 2:1   | 2:1   | 1:1   | 1:1   |
| Inspection:                                         |       |       |       |       |
| Viscosity, SUS—                                     |       |       |       |       |
| at 100° F.                                          | 4,927 | 1,032 | 3,165 | 1,067 |
| at 210° F.                                          | 87.7  | 89.2  | 95.5  | 96.3  |
| Adhesion to metal, percent retained (400 R. P. M.)— |       |       |       |       |
| at 80° F.                                           | 100   | 83    | 100   | 77    |
| at 120° F.                                          | 97    | 77    | 95    | 63    |
| at 160° F.                                          | 97    | 70    | 95    | 57    |

The above data show that cooling without stirring gives products having higher viscosities than products obtained with increased cooling by stirring. It is also to be noted that compositions having a ratio of hydrogenated rosin to polymerized ethylene of 2 to 1 are superior in their metal adhesion characteristics to compositions having a ratio of 1 to 1.

While the above compositions were prepared using a 68-32 blend of 500/3 and 1900/5 Texas oils, equally satisfactory compositions can be obtained by varying the ratio of oils and by using oils of different viscosities. Typical properties of such compositions are as follows:

|                                                     | A     | B     |
|-----------------------------------------------------|-------|-------|
| Composition, percent by wt.:                        |       |       |
| 100/2 Texas oil                                     | 43    | 20    |
| 1900/5 Texas oil                                    | 55    | 78    |
| Hydrogenated rosin                                  | 1.332 | 1.332 |
| Polymerized ethylene                                | 0.668 | 0.668 |
| Ratio of hydrogenated rosin to polymerized ethylene | 2:1   | 2:1   |
| Inspection:                                         |       |       |
| Gravity, °API                                       | 22.0  | 21.1  |
| Viscosity, SUS—                                     |       |       |
| at 100° F.                                          | 728   | 1,535 |
| at 210° F.                                          | 69.0  | 94.5  |
| Viscosity Index                                     | 74    | 64    |
| Flash point, O. C.:°F.                              | 355   | 335   |
| Fire point, O. C.:°F.                               | 405   | 445   |
| Pour point, °F.                                     | -5    | +10   |
| Color, ASTM Union                                   | 4.75  | 5.5   |
| Neutralization Value, ASTM D 974-53T—               |       |       |
| Total Acid No.                                      | 2.1   | 2.1   |
| Ash, percent                                        | 0.012 | 0.012 |

While my invention has been described with reference to various specific examples and embodiments, it will be understood that the invention is not limited to such

examples and embodiments and may be variously practiced within the scope of the claims hereinafter made.

I claim:

1. A lubricating composition consisting essentially of a major proportion of a hydrocarbon oil having a viscosity above about 400 SUS at 100° F. and a minor proportion, sufficient to increase the viscosity of the oil and to impart thixotropic characteristics thereto, of a mixture of hydrogenated rosin of at least about 40 percent saturation and polymerized ethylene having a molecular weight between about 1000 and about 40,000, the weight ratio of hydrogenated rosin to polymerized ethylene being between about 1:3 and about 3:1.

2. A thixotropic lubricating composition consisting essentially of a major proportion of a hydrocarbon oil having a viscosity of about 400 to about 4000 SUS at 100° F., about 0.2 to about 5 percent by weight of polymerized ethylene having a molecular weight between about 1000 and about 40,000, and a hydrogenated rosin of at least about 40 percent saturation, the weight ratio of hydrogenated rosin to polymerized ethylene being between about 1:3 and about 3:1.

3. A thixotropic lubricating composition consisting essentially of a major proportion of a hydrocarbon oil having a viscosity of about 400 to about 4000 SUS at 100° F., about 0.2 to about 5 percent by weight of polymerized ethylene having a molecular weight between about 1000 and about 40,000, and about 0.2 to about 5 percent by weight of a hydrogenated rosin of at least about 40 percent saturation.

4. A thixotropic lubricating composition consisting essentially of a major proportion of a hydrocarbon oil having a viscosity of about 400 to about 4000 SUS at 100° F., about 0.2 to about 5 percent by weight of polymerized ethylene having a molecular weight between about 1000 and about 40,000, and about 0.2 to about 5 percent by weight of a hydrogenated rosin of at least about 40 percent saturation, the weight ratio of hydrogenated rosin to polymerized ethylene being between about 1:3 and about 3:1.

5. A thixotropic lubricating composition consisting essentially of a uniform mixture of about 90 to about 99 percent by weight of a mineral lubricating oil having a viscosity of about 400 to about 4000 SUS at 100° F., about 0.2 to about 5 percent by weight of polymerized ethylene having a molecular weight of about 19,000, and about 0.2 to about 5 percent by weight of a hydrogenated rosin saturated to an extent of about 50 to about 60 percent, the weight ratio of hydrogenated rosin to polymerized ethylene being between about 1:3 and about 3:1.

#### References Cited in the file of this patent

#### UNITED STATES PATENTS

- |    |           |           |                |
|----|-----------|-----------|----------------|
| 70 | 2,221,953 | Read      | Nov. 19, 1940  |
|    | 2,270,319 | Lieber    | Jan. 20, 1942  |
|    | 2,627,938 | Frohmader | Feb. 10, 1953  |
|    | 2,628,187 | Frohmader | Feb. 10, 1953  |
|    | 2,691,647 | Field     | Oct. 12, 1954  |
| 75 | 2,762,775 | Foehr     | Sept. 11, 1956 |